# EUROPEAN PATENT SPECIFICATION

(11) **EP 2 181 212 B1**
(45) Date of publication and mention of the grant of the patent: **23.11.2011**
(21) Application number: 08798455.5
(22) Date of filing: 22.08.2008
(51) Int. Cl.: D01F 6/80, D06P 3/24

(54) **FIBERS COMPRISING COPOLYMERS CONTAINING STRUCTURES DERIVED FROM A PLURALITY OF AMINE MONOMERS INCLUDING 3,3' DIAMINO DIPHENYL SULFONE AND METHODS FOR MAKING SAME**
FASERN AUS COPOLYMEREN MIT AUS MEHREREN AMINMONOMEREN, U. A. 3,3'-DIAMINODIPHENYLSULFON, ABGELEITETEN STRUKTUREN SOWIE VERFAHREN ZU IHRER HERSTELLUNG
FIBRES COMPRENANT DES COPOLYMÈRES INCLUANT DES STRUCTURES DÉRIVÉES D'UNE PLURALITÉ DE MONOMÈRES AMINE COMPRENANT LA 3,3'-DIAMINODIPHÉNYLSULFONE ET PROCÉDÉS DE FABRICATION DE CELLES-CI

(30) Priority: 22.08.2007 US 894913
(43) Date of publication of application: 05.05.2010
(73) Proprietor: E. I. du Pont de Nemours and Company, Wilmington, DE 19898 (US)
(72) Inventor: GABARA, Vlodek, Richmond, Virginia 23238-4804 (US)
(74) Representative: Dannenberger, Oliver Andre
(86) International application number: PCT/US2008/073976
(87) International publication number: WO 2009/026494

(56) References cited:
- DE-A1- 4 411 011
- US-A- 3 287 324
- US-A- 4 072 664
- US-A- 5 174 790
- US-A- 5 667 743

## Description

### FIELD OF THE INVENTION

The invention concerns a fiber, obtainable by spinning a copolymer from the polymerization solution, derived from a plurality of amine monomers, including 3,3'diaminodiphenyl sulfone amine monomer, and at least one acid monomer; and yarns, fabrics and garments comprising this fiber, and methods of making the same. This fiber has use in heat-resistant protective apparel fabrics and garments.

### BACKGROUND OF THE INVENTION

Chinese Patent Publication 1389604A to Wang et al. discloses a fiber known as polysulfonamide fiber (PSA) made by spinning a copolymer solution formed from a mixture of 50 to 95 weight percent 4,4'diaminodiphenyl sulfone and 5 to 50 weight percent 3,3'diaminodiphenyl sulfone copolymerized with equimolar amounts of terephthaloyl chloride in dimethylacetamide.

Chinese Patent Publication 1631941 A to Chen et al. also discloses a method of preparing a PSA copolymer spinning solution formed from a mixture of 4,4'diaminodiphenyl sulfone and 3,3'diaminodiphenyl sulfone in a mass ratio of from 10:90 to 90:10 copolymerized with equimolar amounts of terephthaloyl chloride in dimethylacetamide.

Both these preparations require amine monomers that are diaminodiphenyl sulfones. Unfortunately, diaminodiphenyl sulfones are generally more expensive than other amine monomers and are not widely available and therefore are undesirable as the only types of amine monomers in the copolymer.

United States Patent No. 4,169,932 to Sokolov et al. discloses preparation of poly(paraphenylene) terephthalamide (PPD-T) copolymers using tertiary amines to increase the rate of polycondensation. This patent discloses the PPD-T copolymer may be formed with terephthalic acid dichloride or a mixture of terephthalic acid dichloride (50-95 mole percent) and an aromatic acid dichloride of the diphenyl series (50-5 mole percent). This patent also discloses the PPD-T copolymer can be made by replacing 5 to 50 mole percent of the paraphenylene diamine (PPD) by another aromatic diamine such as 4,4'diaminodiphenyl sulfone, and provides an example of such a copolymer containing 95 mole percent paraphenylene diamine and 5 mole percent 4,4'diaminodiphenyl sulfone. While sulfone monomers can be expensive, one of the benefits of a fiber such as PSA fiber is the quantity of sulfone groups in the polymer chain that make the fiber exceptionally dyeable, something that would not be possible with the high PPD-content polymers of Sokolov.

Therefore, what is needed is a copolymer that is both soluble in nominal organic solvents, has an adequate para-oriented structure for high temperature stability, and also has a high quantity of sulfone groups in the polymer chain.

### SUMMARY OF THE INVENTION

In some embodiments, this invention relates to a fiber comprising a copolymer having a structure derived from the reaction of a plurality of amine monomers and an acid monomer, wherein the plurality of amine monomers consists essentially of 3,3 diaminodiphenyl sulfone and a monomer having the structure

H₂N Ar₁-NH₂

the 3,3'diaminodiphenyl sulfone being at least 25 mole percent of the total amount of amine monomers; and at least one acid monomer has a structure of

Cl-CO-Ar₂-CO-Cl

the aromatic group Ar₁ being any unsubstituted or substituted para-oriented benzene ring and Ar₂ being any unsubstituted or substituted aromatic ring structure being the same as or different from Ar₁. This invention further relates to a flame-resistant yarn, a fabric, and a protective garment comprising the above fiber.

This invention further describes a method of producing a fiber comprising the steps of a) forming a copolymer by reacting a plurality of amine monomers and one or more acid monomers, wherein the plurality of amine monomers consists essentially of 3,3'diaminodiphenyl sulfone and a monomer having the structure

H₂N- Ar₁-NH₂

the 3,3'diaminodiphenyl sulfone being at least 25 mole percent of the total amount of amine monomers; and at least one acid monomer having a structure of

Cl-CO-Ar₂-CO-Cl

the aromatic group Ar₁ being any unsubstituted or substituted para-oriented benzene ring and Ar₂ being any unsubstituted or substituted aromatic ring structure being the same as or different from Ar₁;
b) providing the copolymer in a solution suitable for spinning fibers; and
c) spinning fibers from the copolymer solution.

### DETAILED DESCRIPTION

The invention concerns a fiber, obtainable by spinning a copolymer from the polymerization solution, derived from 3,3'diaminodiphenyl sulfone amine monomer, at least one other amine monomer, and one or more acid monomers. In some preferred embodiments the fiber is a flame-resistant fiber having limiting oxygen index of 21 or greater. By "flame resistant" it is meant the spun staple yarn, or fabrics made from the yarn, will not support a flame in air. In preferred embodiments the fabrics have a limiting oxygen index (LOI) of about 26 and higher.

For purposed herein, the term "fiber" is defined as a relatively flexible, macroscopically homogeneous body having a high ratio of length to the width of the cross-sectional area perpendicular to that length. The fiber cross section can be any shape, but is typically round. Herein, the term "filament" or "continuous filament" is used interchangeably with the term "fiber."

As used herein, the term "staple fibers" refers to fibers that are cut to a desired length or are stretch broken, or fibers that occur naturally with or are made having a low ratio of length to the width of the cross-sectional area perpendicular to that length when compared with filaments. Man made staple fibers are cut or made to a length suitable for processing on cotton, woolen, or worsted yarn spinning equipment. The staple fibers can have (a) substantially uniform length, (b) variable or random length, or (c) subsets of the staple fibers have substantially uniform length and the staple fibers in the other subsets have different lengths, with the staple fibers in the subsets mixed together forming a substantially uniform distribution.

In some embodiments, suitable staple fibers have a length of about 0.25 centimeters (0.1 inches) to about 30 centimeters (12 inches). In some embodiments, the length of a staple fiber is from about 1 cm (0.39 in) to about 20 cm (8 in). In some preferred embodiments the staple fibers made by short staple processes have a staple fiber length of about 1 cm (0.39 in) to about 6 cm (2.4 in). The term continuous filament refers to a flexible fiber having relatively small-diameter and whose length is longer than those indicated for staple fibers.

By copolymer fibers having a structure derived from the amine monomer 3,3'diaminodiphenyl sulfone, it is meant the copolymer was made from a monomer generally having the structure:

NH₂-Ar-SO₂-Ar-NH₂

wherein Ar is any unsubstituted or substituted six-membered aromatic group of carbon atoms having para-oriented linkages with the SO₂ group. In one preferred embodiment Ar is an unsubstituted benzyl ring. The copolymer has mixture of amine monomers, of which at least 25 mole percent is 3,3'diaminodiphenyl sulfone to help provide adequate dyeability and solubility in organic solvents. At least one other amine monomer present in the copolymer has the general structure:

H₂N-Ar₁-NH₂

wherein Ar₁ is any unsubstituted or substituted a para-oriented benzene ring. The para-oriented aromatic ring structure provides the copolymer with high temperature stability, and one preferred amine monomer is paraphenylene diamine. In one embodiment substantially all (95 mole percent or greater) of the amine monomers that are not 3,3'diaminodiphenyl sulfone are derived from para-oriented structures.

In some other embodiments, the plurality of amine monomers has 25 to 45 mole percent 3,3'diaminodiphenyl sulfone and 55 to 75 mole percent of another amine monomer containing the aromatic group Ar₁.

The amine monomers are copolymerized with at least one acid monomer in a compatible solvent to create a copolymer. The acid monomers have the structure

Cl-CO-Ar₂-CO-Cl

wherein Ar₂ is any unsubstituted or substituted aromatic ring structures and is the same as or different from Ar₁, however, if they are the same, they have different linkage orientation in the structure. In some preferred embodiments Ar₁ and Ar₂ are both unsubstituted six-membered aromatic groups of carbon atoms and the aromatic group Ar₁ has *para*-oriented linkages and aromatic group Ar₂ has *meta-*oriented linkages. For example, Ar₁ and Ar₂ can be both benzene rings while Ar₁ can be a benzene ring having *para*-oriented linkages while Ar₂ has *meta*-oriented linkages. Examples of useful monomers include terephthaloyl chloride, isophthaloyl chloride, and the like, with terephthaloyl chloride being a preferred monomer.

In one preferred embodiment, more than one acid monomer is used with the combination of terephthaloyl chloride and isophthaloyl chloride being one preferred combination. In some embodiments, the plurality of acid monomers includes 55 to 95 mole percent of acid monomers having *para*-oriented aromatic groups, such as terephthaloyl chloride, and 5 to 45 mole percent acid monomers having *meta*-oriented aromatic groups, such as isophthaloyl chloride.

It is believed that at least 15 percent of the total amount of aromatic monomers used to make the copolymer should contain monomers having meta-oriented functionality in order for the final copolymer to be soluble in the polymerization solvent and suitable for spinning fibers. By "total amount of aromatic monomers" is meant the total of all amine monomers and acid monomers added together. In other words, if the mixture of acid monomers contains only 15 mole percent of acid monomers having meta-oriented aromatic groups, at least 15 mole percent of the amine monomers must have meta-oriented aromatic groups, to make the total amount of aromatic monomers used to be 15 percent; based on a 1-to-1 amine-acid stoichiometry. In some embodiments 20 to 30 percent of the total amount of aromatic monomers used to make the copolymer contain monomers having meta-oriented functionality. In some embodiments, the maximum amount of monomers having para-oriented functionality is 85 percent of the total amount of aromatic monomers used to make the copolymer.

In a one embodiment, these fiber having a limiting oxygen index (LOI) of 21 or greater, meaning the fiber or fabrics made solely from the fiber will not support a flame in air. In some preferred embodiments the textile staple fiber has a LOI of at least 26 or greater.

In some embodiments the fiber has a break tenacity of at least 3 grams per denier 26.49 mN ((2.7 grams) per dtex) or greater, and in some preferred embodiments the fiber has a break tenacity of at least 4 grams per denier 35.32 mN (3.6 grams) per dtex) or greater.

Fabrics can be made from the fibers, or from spun staple yarns or multifilament continuous yarns comprising the fibers, and such fabrics can include but are not limited to woven or knitted fabrics. Such fabrics are well known to those skilled in the art. By "woven" fabric is meant a fabric usually formed on a loom by interlacing warp or lengthwise yarns and filling or crosswise yarns with each other to generate any fabric weave, such as plain weave, crowfoot weave, basket weave, satin weave, twill weave, and the like. Plain and twill weaves are believed to be the most common weaves used in the trade and are preferred in many embodiments.

By "knitted" fabric is meant a fabric usually formed by interlooping yarn loops by the use of needles. In many instances, to make a knitted fabric spun staple yarn is fed to a knitting machine which converts the yarn to fabric. If desired, multiple ends or yarns can be supplied to the knitting machine either plied of unplied; that is, a bundle of yarns or a bundle of plied yarns can be co-fed to the knitting machine and knitted into a fabric, or directly into a article of apparel such as a glove, using conventional techniques. In some embodiments it is desirable to add functionality to the knitted fabric by co-feeding one or more other staple or continuous filament yarns with one or more spun staple yarns having the intimate blend of fibers. The tightness of the knit can be adjusted to meet any specific need. A very effective combination of properties for protective apparel has been found in for example, single jersey knit and terry knit patterns.

In some particularly useful embodiments, the fibers and yarns containing the fibers can be used to make flame-resistant garments. In some embodiments the garments can have essentially one layer of the protective fabric made from the spun staple yarn. Exemplary garments of this type include jumpsuits and coveralls for fire fighters or for military personnel. Such suits are typically used over the firefighters clothing and can be used to parachute into an area to fight a forest fire. Other garments can include pants, shirts, gloves, sleeves and the like that can be worn in situations such as chemical processing industries or industrial electrical/utility where an extreme thermal event might occur. In some preferred embodiments the fabrics have an arc resistance of at least 0.099 joules per square centimeter per grams per square meter (0.8 calories per square centimeter per ounce per square yard).

In other embodiments the fibers and yarns containing the fibers can be used in any layer of multilayer flame-resistant garments having a general construction such as disclosed in United States Patent No. 5,468,537. Such garments generally have three layers or three types of fabric constructions, each layer or fabric construction performing a distinct function. There is an outer shell fabric that provides flame protection and serves as a primary defense from flames for the fire fighter. Adjacent the outer shell is a moisture barrier that is typically a liquid barrier but can be selected such that it allows moisture vapor to past through the barrier. Laminates of Gore-Tex® PTFE membrane or Neoprene® membranes on a fibrous nonwoven or woven meta-aramid scrim fabric are moisture barriers typically used in such constructions. Adjacent the moisture barrier is a thermal liner, which generally includes a batt of heat resistant fiber attached to an internal face cloth. The moisture barrier keeps the thermal liner dry and thermal liner protects the wearer from heat stress from the fire or heat threat being addressed by the wearer.

This invention further describes a method of producing a fiber comprising the steps of a) forming a copolymer by reacting a plurality of amine monomers and one or more acid monomers, wherein the plurality of amine monomers consists essentially of 3,3'diaminodiphenyl sulfone and at least one monomer having the structure

H₂N- Ar₁-NH₂

the 4,4'diaminodiphenyl sulfone being at least 25 mole percent of the total amount of amine monomers; and at least one acid monomer having a structure of

Cl-CO-Ar₂-CO-Cl

the aromatic group Ar₁ being any unsubstituted or substituted para-oriented benzene ring; b) providing the copolymer in a solution suitable for spinning fibers; and c)spinning fibers from the copolymer solution.

In one embodiment, the polymer and copolymer derived from a sulfone monomer can preferably be made via polycondensation of one or more types of diamine monomer with one or more types of chloride monomers in a dialkyl amide solvent such as N-methyl pyrrolidone, dimethyl acetamide, or mixtures thereof. In some embodiments of the polymerizations of this type an inorganic salt such as lithium chloride or calcium chloride is also present. If desired the polymer can be isolated by precipitation with non-solvent such as water, neutralized, washed, and dried. The general polymerization techniques disclosed in Chinese Patent Publications 1389604A to Wang et al. and 1631941A to Chen et al. can be applied to these solutions, and if desired the techniques disclosed in United States Patent No. 4,169,932 to Sokolov et al. can also be followed. The polymer can also be made via interfacial polymerization which produces polymer powder directly that can then be dissolved in a solvent for fiber production.

The polymer or copolymer can be spun into fibers via solution spinning, using a solution of the polymer or copolymer in either the polymerization solvent or another solvent for the polymer or copolymer. Fiber spinning can be accomplished through a multi-hole spinneret by dry spinning, wet spinning, or dry-jet wet spinning (also known as air-gap spinning) to create a multi-filament yarn or tow as is known in the art. The fibers in the multi-filament yarn or tow after spinning can then be treated to neutralize, wash, dry, or heat treat the fibers as needed using conventional technique to make stable and useful fibers. Exemplary dry, wet, and dry-jet wet spinning processes are disclosed U.S. Patent Nos. 3,063,966; 3,227,793; 3,287,324; 3,414,645; 3,869,430; 3,869,429; 3,767,756; and 5,667,743.

Continuous filament fibers and multifilament yarns of continuous filaments can be made by processes well known to those skilled in the art. For example, multifilament continuous filament yarns can be made by winding filament threadlines directly on a bobbin, with or without twist; or if needed, combining multiple filament threadlines to form higher denier yarns.

Alternatively, continuous filament can be converted into staple fiber by any number of ways known in the art, including processes that creel a number of bobbins of continuous filaments and concurrently cut the filaments to form cut staple fibers. For example, the staple fibers can be cut from continuous straight fibers using a rotary cutter or a guillotine cutter resulting in straight (i.e., non crimped) staple fiber, or additionally cut from crimped continuous fibers having a saw tooth shaped crimp along the length of the staple fiber, with a crimp (or repeating bend) frequency of preferably no more than 8 crimps per centimeter.

The staple fibers can also be formed by stretch breaking continuous fibers resulting in staple fibers with deformed sections that act as crimps. Stretch broken staple fibers can be made by breaking a tow or a bundle of continuous filaments during a stretch break operation having one or more break zones that are a prescribed distance creating a random variable mass of fibers having an average cut length controlled by break zone adjustment.

Generally these staple fibers are formed into bales; the staple fibers are then formed into spun staple yarns by processes that involve first opening the bales of staple fibers and then further processing the clumps of staple fibers in openers, blenders, and cards to form slivers of staple fibers. Generally, in the individual staple fibers are opened or separated to a degree that is normal in fiber processing to make a useful fabric, such that fiber knots or slubs and other major defects due to poor opening of the staple fibers are not present in an amount that detract from the final fabric quality. A carding machine is commonly used to separate, align, and deliver fibers into a continuous strand of loosely assembled fibers without substantial twist, commonly known as carded sliver. The carded sliver is processed into drawn sliver, typically by, but not limited to, a two-step drawing process.

Spun staple yarns are then formed from the drawn sliver using conventional techniques. These techniques include conventional cotton system, short-staple spinning processes, such as, for example, open-end spinning, ring-spinning, or higher speed air spinning techniques such as Murata air-jet spinning where air is used to twist the staple fibers into a yam. The formation of spun yarns useful in fabrics can also be achieved by use of conventional woolen systems, long-staple or stretch-break spinning processes, such as, for example, worsted or semi-worsted ring-spinning.

Regardless of the processing system, ring-spinning is the generally preferred method for making the spun staple yarns using traditional long and short staple ring spinning processes that are well known in the art. For short staple, cotton system spinning fiber lengths from about 1.9 to 5.7 cm (0.75 in to 2.25 in) are typically used. For long staple, worsted or woolen system spinning, fibers up to about 16.5 cm (6.5 in) are typically used.

Spun staple yarns can also be made directly by stretch breaking using stretch-broken tow to top staple processes. The staple fibers in the yarns formed by traditional stretch break processes typically have length of up to about 18 cm (7 in) long. However spun staple yarns made by stretch breaking can also have staple fibers having maximum lengths of up to around 50 cm (20 in.) through processes as described for example in PCT Patent Application No. WO 0077283. Stretch broken staple fibers normally do not require crimp because the stretch-breaking process imparts a degree of crimp into the fiber.

### TEST METHODS

Basis weight values were obtained according to FTMS 191A; 5041.

Arc Resistance Test. The arc resistance of fabrics is determined in accordance with ASTM F-1959-99 "Standard Test Method for Determining the Arc Thermal Performance Value of Materials for Clothing". The Arc Thermal Performance Value (ATPV) of each fabric, which is a measure of the amount of energy that a person wearing that fabric could be exposed to that would be equivalent to a 2nd degree bum from such exposure 50% of the time.

Grab Test. The grab resistance of fabrics (the break tensile strength) is determined in accordance with ASTM D-5034-95 "Standard Test Method for Breaking Strength and Elongation of Fabrics (Grab Test)".

Thermal Protection Performance (TPP) Test. The thermal protection performance of fabrics is determined in accordance with NFPA 2112 "Standard on Flame Resistant Garments for Protection of Industrial Personnel Against Flash Fire". The thermal protective performance relates to a fabric's ability to provide continuous and reliable protection to a wearer's skin beneath a fabric when the fabric is exposed to a direct flame or radiant heat.

Vertical Flame Test. The char length of fabrics is determined in accordance with ASTM D-6413-99 "Standard Test Method for Flame Resistance of Textiles (Vertical Method)".

Limiting Oxygen Index (LOI) is the minimum concentration of oxygen, expressed as a volume percent, in a mixture of oxygen and nitrogen that will just support the flaming combustion of a material initially at room temperature under the conditions of ASTM G125 / D2863.

### Examples

The invention is illustrated by, but is not intended to be limited by the following examples:

### Example 1

The solvent dimethyl acetamide is purified and dried before use by distillation in the presence of P₂O₅- 200 grams of this solvent is placed in a flask equipped with a mechanical stirrer and a nitrogen inlet 9.92 grams of 3,3'-diaminodiphenyl sulfone and 6.49 grams of paraphenylene diamine are dissolved in the solvent to form a roughly 60/40 molar solution and the solution is cooled to 0° C by water/ice bath. 20.3 grams of terephthaloyl chloride is added to the flask with agitation. The cooling bath is removed and the polymerization is continued for 30 minutes. At that point 7.4 grams of calcium hydroxide is added to neutralize HCl which is a byproduct of the polymerization. The resulting material is a viscous solution that is spun into fibers and the fibers are processed into fabrics and garments.

### Comparative Example A

Example 1 is repeated, except 3.28 grams of 3,3'-diaminodiphenyl sulfone and 13.13 grams of paraphenylene diamine were used to make a 20/80 molar solution. Upon addition of the terephthaloyl chloride, the polymer precipitates in a gel like form, making a mixture that is not capable of being spun into fibers.

### Example 2

Example 1 is repeated except that the solvent dimethyl acetamide is replaced with N-methyl pyrrolidone without changes in the procedure. A viscous copolymer solution results that after degassing is used to form fibers that are subsequently processed into fabrics and garments.

### Example 3

Example 1 is repeated except that the single acid monomer terephthaloyl chloride is replaced by first forming a mixture of isophthaloyl chloride (ICL) and terephthaloyl chloride (TCL), the amount of ICL being 25 parts by weight and the TCL amount being 75 parts by weight based on the total weight of the acid monomer added in Example 1, and then adding this mixture to the flask with agitation. A viscous copolymer solution results that after degassing is used to form fibers that are subsequently processed into fabrics and garments.

### Example 4

Example 3 is repeated except that 45 parts by weight of ICL and 55 parts by weight TCL are used based on the total weight of the acid monomer added in Example 3, and the acid chlorides are not first mixed but added separately to the flask with agitation. A viscous copolymer solution results that after degassing is used to form fibers that are subsequently processed into fabrics and garments.

### Example 5

A thermally protective and durable fabric is prepared having in both the warp and fill ring spun yarns comprising a staple fiber of the process of Example 1. A sliver is prepared and is processed by the conventional cotton system equipment and is then spun into a spun staple yarn having twist multiplier 4.0 and a single yarn size of about 21 tex (28 cotton count) using a ring spinning frame. Two single yarns are then plied on a plying machine to make a flame resistant two-ply warp yam. Using a similar process and the same twist a 24 tex (24 cotton count) yarn is made for use in the fill. As before, two of these single yarns are plied to form a flame resistant two-ply fill yarn.

The yarns are then used as the warp and fill yarns and are woven into a fabric on a shuttle loom, making a greige fabric having a 2x1 twill weave and a construction of 26 ends x 17 picks per cm (72 ends x 52 picks per inch), and a basis weight of about 215 g/m² (6.5 oz/yd²). The greige twill fabric is then scoured in hot water and is dried under low tension. The scoured fabric is then jet dyed using basic dye. The finished fabric has a basis weight of about 231 g/m² (7 oz/yd²). The fabrics are used to make protective garments suitable for people who work near flames or high temperatures.

## Claims

1. A fiber comprising a copolymer having a structure derived from the reaction of a plurality of amine monomers and an acid monomer, wherein
i) the plurality of amine monomers consists essentially of 3,3'diaminodiphenyl sulfone and a monomer having the structure
H₂N- Ar₁-NH₂,
the 3,3'diaminodiphenyl sulfone being at least 25 mole percent of the total amount of amine monomers; and
ii) at least one acid monomer has a structure of
Cl-CO-Ar₂-CO-Cl,
the aromatic group Ar₁ being any unsubstituted or substituted para-oriented benzene ring, and Ar₂ being any unsubstituted or substituted aromatic ring structure being the same as or different from Ar₁.

2. The fiber of claim 1 wherein the amine monomer containing the aromatic group Ar₁ is paraphenylene diamine.

3. The fiber of claim 1 wherein the plurality of amine monomers has 25 to 45 mole percent 3,3'diaminodiphenyl sulfone and 55 to 75 mole percent of the amine monomer containing the aromatic group Ar₁.

4. The fiber of claim 1 wherein the aromatic group Ar₂ is a meta-oriented benzene ring.

5. The fiber of claim 1 wherein the acid monomer is selected from the group consisting of terephthaloyl chloride, isophthaloyl chloride, and mixtures thereof.

6. The fiber of claim 1 wherein the amine monomer containing the aromatic group Ar₁ is paraphenylene diamine and the acid monomer is a mixture of terephthaloyl chloride and isophthaloyl chloride.

7. The fiber of claim 1 comprising a first acid monomer present in 55 to 95 parts by weight and a second acid monomer present in 5 to 45 parts by weight, based on the total amount of those two monomers.

8. A flame-resistant yarn comprising the fiber of claim 1.

9. The flame-resistant yarn of claim 8 wherein the fiber is present in the yarn as a continuous filament.

10. The flame-resistant yarn of claim 8 wherein the fiber is present in the yarn as a staple fiber

11. A fabric comprising the fiber of claim 1.

12. A protective garment comprising the fiber of claim 1.

## Patentansprüche

1. Faser umfassend ein Copolymer, das eine Struktur aufweist, die aus der Reaktion einer Vielzahl von Aminmonomeren und einem sauren Monomer stammt, wobei
i) die Vielzahl von Aminmonomeren im Wesentlichen aus 3,3'-Diaminodiphenylsulfon und einem Monomer, das die Struktur H₂N-Ar₁-NH₂ aufweist, besteht, wobei das 3,3'-Diaminodiphenylsulfon mindestens 25 Molprozent der Gesamtmenge von Aminmonomeren ausmacht; und
ii) mindestens ein saures Monomer die Struktur Cl-CO-Ar₂-CO-Cl aufweist, wobei die aromatische Gruppe Ar₁ irgendein unsubstituierter oder substituierter paraorientierter Benzolring ist und Ar₂ irgendeine unsubstituierte oder substituierte aromatische Ringstruktur ist, die gleich wie oder verschieden von Ar₁ ist.

2. Faser nach Anspruch 1, wobei das Aminmonomer, das die aromatische Gruppe Ar₁ enthält, Paraphenylendiamin ist.

3. Faser nach Anspruch 1, wobei die Vielzahl von Aminmonomeren 25 bis 45 Molprozent 3,3'-Diaminodiphenylsulfon und 55 bis 75 Molprozent des Aminmonomers aufweist, das die aromatische Gruppe Ar₁ enthält.

4. Faser nach Anspruch 1, wobei die aromatischen Gruppe Ar₂ ein meta-orientierter Benzolring ist.

5. Faser nach Anspruch 1, wobei das saure Monomer aus der Gruppe ausgewählt ist bestehend aus Terephthaloylchlorid, Isophthaloylchlorid und Mischungen davon.

6. Faser nach Anspruch 1, wobei das Aminmonomer, das die aromatische Gruppe Ar₁ enthält, Paraphenylendiamin ist und das saure Monomer eine Mischung von Terephthaloylchlorid und Isophthaloylchlorid ist.

7. Faser nach Anspruch 1, umfassend ein erstes saures Monomer, das in einer Menge von 55 bis 95 Gewichtsteilen vorliegt, und ein zweites saures Monomer, das in einer Menge von 5 bis 45 Gewichtsteilen, auf die Gesamtmenge dieser beiden Monomere bezogen, vorliegt.

8. Flammwidriges Garn umfassend die Faser nach Anspruch 1.

9. Flammwidriges Garn nach Anspruch 8, wobei die Faser in dem Garn als Endlosfaser vorliegt.

10. Flammwidriges Garn nach Anspruch 8, wobei die Faser in dem Garn als Stapelfaser vorliegt.

11. Textilstoff umfassend die Faser nach Anspruch 1.

12. Schutzkleidung umfassend die Faser nach Anspruch 1.

## Revendications

1. Fibre comprenant un copolymère ayant une structure dérivée de la réaction d'une pluralité de monomères d'amine et d'un monomère d'acide, dans laquelle
i) la pluralité des monomères d'amine est essentiellement constituée de 3,3'-diaminodiphényl sulfone et d'un monomère ayant la structure H₂N-Ar₁-NH₂, la 3,3'-diaminodiphényl sulfone étant au moins de 25 pour cent en mole de la quantité totale des monomères d'amine; et
ii) au moins un monomère d'acide a une structure de Cl-CO-Ar₂-CO-Cl, le groupe aromatique Ar₁ étant n'importe quel cycle benzénique non substitué ou substitué orienté en position para, et Ar₂ étant n'importe quelle structure cyclique aromatique non substituée ou substituée étant identique ou différente de Ar₁.

2. Fibre selon la revendication 1, dans laquelle le monomère d'amine contenant le groupe aromatique Ar₁ est de la paraphénylène diamine.

3. Fibre selon la revendication 1, dans laquelle la pluralité des monomères d'amine a 25 à 45 pour cent en mole de 3,3'-diaminodiphényl sulfone et 55 à 75 pour cent en mole du monomère d'amine contenant le groupe aromatique Ar₁.

4. Fibre selon la revendication 1, dans laquelle le groupe aromatique Ar₂ est un cycle benzénique orienté en position méta.

5. Fibre selon la revendication 1, dans laquelle le monomère d'acide est choisi parmi le groupe constitué du chlorure de téréphtaloyle, du chlorure d'isophtaloyle, et des mélanges de ceux-ci.

6. Fibre selon la revendication 1, dans laquelle le monomère d'amine contenant le groupe aromatique Ar₁ est la paraphénylène diamine et le monomère d'acide est un mélange de chlorure de téréphtaloyle et de chlorure d'isophtaloyle.

7. Fibre selon la revendication 1, comprenant un premier monomère d'acide présent en 55 à 95 parties en poids et un second monomère d'acide présent en 5 à 45 parties en poids, basées sur la quantité totale de ces deux monomères.

8. Fil résistant aux flammes comprenant la fibre selon la revendication 1.

9. Fil résistant aux flammes selon la revendication 8, dans lequel la fibre est présente dans le fil sous la forme d'un filament continu.

10. Fil résistant aux flammes selon la revendication 8, dans lequel la fibre est présente dans le fil sous la forme d'une fibre discontinue.

11. Textile comprenant la fibre selon la revendication 1.

12. Vêtement protecteur comprenant la fibre selon la revendication 1.
